# EUROPEAN PATENT SPECIFICATION

(11) **EP 0 070 709 B1**
(45) Date of publication and mention of the grant of the patent: **01.10.1986**
(21) Application number: 82303749.4
(22) Date of filing: 16.07.1982
(51) Int. Cl.: D01F 1/10, D01F 6/90, D21F 7/08

(54) **Mineral filled abrasion-resistant monofilament**
Abriebfestes, einen Mineralfüllstoff enthaltendes Monofilament
Monofilament résistant à l'abrasion et contenant une charge minérale

(30) Priority: 17.07.1981 US 283905
(43) Date of publication of application: 26.01.1983
(73) Proprietor: E.I. DU PONT DE NEMOURS AND COMPANY, Wilmington Delaware 19898 (US)
(72) Inventor: Bond, William Bradford, Marietta Ohio 45750 (US); Gall, Walter George, Tucson Arizona 85704 (US); Saxton, Ronald Luther, West Grove Pennsylvania 19390 (US)
(74) Representative: Woodman, Derek

## Description

### Background of the Invention

In the preparation of paper, woven support belts are used for the initial casting and subsequent treatment of the paper. These belts are known as paper clothing. A variety of materials has been used in the manufacture of such belts, including metals, and, more recently, thermoplastic monofilaments. Thermoplastic materials which have been used in the weaving of these belts include nylon as well as polyester monofilaments.

A particularly satisfactory combination of materials for paper clothing is a polyester monofilament, woven in the machine direction of the belt, with transverse monofilaments composed either partly or entirely of a polyamide monofilament. Particularly in such applications, a need exists for a polyamide monofilament having improved resistance to abrasion when the abrasive force is applied transversely to the longitudinal dimension of the monofilament.

US-A-3397171 discloses polyamide textile fibers containing kaolinite but does not disclose incorporating kaolinite in monofilaments having diameters greater than 2 mils (50.8 pm).

### Summary of the Invention

The present invention provides a polyamide monofilament which exhibits outstanding resistance to abrasive forces applied transversely to the longitudinal dimension of the monofilament.

Specifically, the instant invention provides an oriented polyamide monofilament having a diameter of from 5 to 30 mils (127 to 762 pm) and comprising fiber or filament-forming polyamide and about from 2 to 20 weight percent, based on the total weight of the monofilament, of aluminum silicate having an average particle size of about from 1 to 8 µm.

The instant invention further provides, a woven, heat set, papermaking belt with machine and transverse direction thermoplastic filaments, characterised in that at least about 25% of the filaments in the transverse direction are monofilaments having a diameter of from 5 to 30 mils (127 to 762 µm) and comprising filament forming polyamide and about from 2 to 20 weight percent, based on the total weight of the filament of an aluminum silicate having an average particle size of about from 1 to 8 um.

### Detailed Description of the Invention

The polyamides used for preparation of the oriented monofilaments of the present invention are noncyclic polyamides of fiber-forming molecular weight having relative viscosity generally between 25 and 150 as determined by ASTM D-789-62T. These polyamides include, for example, polycaprolactam (6 nylon), polyhexamethylene adipamide (66 nylon), polyhexamethylene decanoamide (610 nylon), and polyhexamethylene dodecanoamide (612 nylon). Polyamide copolymers and polymer blends can also be used, such as those prepared from 6 nylon and 66 nylon. Of these, polyhexamethylene adipamide (66 nylon) and polyhexamethylene dodecanoamide (612 nylon) have been found to be paticularly satisfactory for use in paper clothing.

In accordance with the present invention, about from 2 to 20 weight percent, and preferably about from 4 to 10 weight percent, of aluminum silicate is blended with the polyamide used for the preparation of the monofilaments. Less than about 2 weight percent of the aluminum silicate does not provide the markedly improved transverse direction abrasion resistance of the present invention, while quantities of aluminum silicate in excess of 20 weight percent of the monofilament unnecessarily weaken the filament with no further beneficial effects.

The aluminum silicate used in the present invention should be of the type generally commercially available in a uniform particulate configuration. The aluminum silicate should have a particle size such that 90% by weight or more of the particles are less than 15 µm and the average particle size is about from 1 to 8 pm. Particularly satisfactory aluminum silicate clays are those in which 98% of the particles are less than 10 pm and have an average particle size of about from 1 to 6 pm. Aluminum silicates of this type are described in detail in United States Patent 3,419,517, and are commercially available as Satinton^{®} from Engelhard Minerals and Chemicals Corp. of Edison, New Jersey.

The products of the present invention are preferably prepared by combining the nylon polymer with a coupling agent prior to the incorporation of the aluminum silicate. The incorporation of the coupling agent provides improved adhesion of the aluminum silicate to the nylon. Coupling agents which can be used include those organosilane and phosphorus coupling agents described in Miller U.S. Patents 3,344,107, 3,471,435 and 3,488,319.

In a preferred embodiment of the present invention, the monofilaments further comprise about from 0.5 to 10 weight percent of an ethylene copolymer having a Melt Index of about from 0.3 to 30. At least about 50% of the ethylene copolymer should be a graft copolymer prepared from (a) a backbone of polymer selected from the group consisting of thermoplastic polymers of ethylene and copolymers derived from ethylene and C₃-C₈ alpha-olefins and (b) a graft monomer selected from the group consisting of unsaturated carboxylic acids, anhydrides and dianhydrides. Less than 1.0 weight percent of this ethylene copolymer additive provides little or no appreciable improvement in abrasion resistance for the finished monofilament, while quantities in excess of 10 weight percent result in a drop in tensile strength for the monofilament. Particularly outstanding improvement in monofilament characteristics is realized through the use of about from 1.2 to 5 weight percent of the graft copolymer.

The graπ copoiymer, when used, should have a Melt Index of about from 0.3 to 30. Ethylene polymers having a Melt Index outside of this range can result in processing difficulties. Particularly satisfactory are those graft copolymers having a Melt Index of about from 0.5 to 20.

Melt Index is measured according to ASTM D―1238―79, condition E. In that test, the rate of extrusion in grams per 10 minutes [through an orifice 0.0825 inch (0.210 cm) in diameter and 0.315 inch (0.800 cm) in length] is determined for the material under test at 190°C and under the force of a piston having a diameter of 0.373 inch (0.947 cm) and a total weight of 2,160 grams.

Polymeric materials which can be used as a backbone polymer in the graft copolymers are generally selected from thermoplastic polymers of ethylene and copolymers derived from ethylene and C₃-Cg alpha-olefins. Backbone polymers which are substantially saturated include polymers of ethylene and copolymers derived from ethylene and alpha-olefins. Backbone polymers which exhibit unsaturation include those having a substantially saturated backbone chain with unsaturated side chains, including copolymers derived from ethylene and alpha-olefins. The term alpha-olefin includes monoolefins and diolefins and does not include ethylene.

Graft monomers which can be used for the preparation of the graft copolymer additives of the present invention include unsaturated carboxylic acids, anhydrides and dianhydrides thermally stable at the temperature of the grafting reaction. Graft monomers which can be used for the preparation of these additives include methacrylic acid; acrylic acid; glycidyl methacrylate; 2-hydroxy ethylacrylate; 2-hydroxy ethyl methacrylate; diethyl maleate, monoethyl maleate; di-n-butyl maleate; maleic anhydride; maleic acid; fumaric acid; itaconic acid; dodecenyl succinic anhydride; 5-norbornene-2,3-anhydride; and nadic anhydride (3,6-endomethylene-1,2,3,6-tetrahydrophthalic anhydride).

The graft copolymers can be prepared by a variety of reaction techniques. However, particularly preferred is that process described in Flexman, Jr. et al. U.S. Patent 4,026,967, wherein the reaction of the components is conducted in baffled tubular reactors which exhibit dispersed plug flow character and which provide rapid heating and cooling of reactants, short reaction time with uniform material residence time, and radial uniformity of temperature. In general, the graft comonomers can comprise about from 0.15 to 2.0 weight percent of the graft copolymer. A graft copolymer found to be particularly satisfactory in the invention is that prepared from polyethylene having a density of about from 0.94 to 0.97 g/cm³ and grafted with about from 0.15 to 0.75 weight percent graft monomer, and especially furmaric acid or maleic anhydride monomers.

The blending of the components of the monofilament can be carried out in any sequence convenient to the particular manufacturing operation involved. However, in general, it has been found convenient to prepare concentrates of each additive in nylon prior to final blending to aid in the accurate measurement of each of the components.

After blending of the components, the monofilaments are prepared according to customary techniques. The molten nylon, blended with the aluminum silicate and any other additives, is extruded through a die into a quench medium, after which it is oriented. The monofilaments should be oriented about from 3.4 to 6.0 times their original length, and preferably about from 3.5 to 4.7 times their original length. In general, the diameter of the final monofilament should be about from 5 to 30 mils (127 to 762 pm), and preferably about from 10 to 20 mils (254 to 508 pm).

The monofilaments of the present invention can be woven into papermaking belts according to conventional weaving techniques. The type and density of the weave will, of course, depend on the type of paper and papermaking operation for which the belt is to be used. The present monofilaments are particularly satisfactory when used in combination with polyester monofilaments in a woven belt in which the polyester monofilaments make up the machine direction strands and the monofilaments of the present invention comprise at least about 25%, and preferably about from 25% to 50% of the transverse direction strands.

After weaving, the papermaking belts are heat set according to conventional techniques to stabilize the weave. Typical heat setting conditions will vary with the polymer, filaments, diameter and weave, but will typically involve heating under tension in a hot air oven for about from 15 minutes to 1 hour at a temperature of about from 300 to 400°F (149 to 204°C).

The improved monofilaments of the present invention, when used as transverse direction strands in papermaking belts, exhibit excellent resistance to the transverse direction abrasion encountered in belts of this type. This abrasion resistance permits improved operation for apparatus using such belts, in that the period between belt replacements is increased significantly.

The present invention is further illustrated in the following examples, in which parts and percentages are by weight unless otherwise indicated.

### Examples 1-9 and Comparative Examples A-D

A concentrate of aluminum silicate and nylon 612 was prepared by tumbling 12 pounds (5.44 Kg) of nylon 612 for 30 minutes with 50 grams of gamma-aminopropyl triethoxy silane coupling agent. Eight pounds (3.63 Kg) of aluminum silicate of 1.3 um particle size was added and tumbled for an additional 30 minutes. The blend was then extruded in a 53 mm twin-screw extruder at 150 pph (68.1 Kg/h), with a screw speed of 200 rpm and a barrel temperature of from 250 to 265°C under full vacuum at the vent port. The resulting strands were water quenched and cut into flake.

Next, concentrates were prepared of nylon 612 with three ethylene copolymers, designated Additives A, B and C. Additive A was a graft copolymer having a Melt Index of 11.4 and an average anhydride graft level of 0.4%. Additive B was also a graft copolymer having a Melt Index of 0.59 and an average anhydride graft level of 1.75%. Additive C was an ungrafted ethylene-a-olefin copolymer having a melt flow of 1.0 g in 10 minutes at 280°C with a 5000 g load and the same orifice dimensions used in the Melt Index method.

Nylon 612 having an inherent viscosity of 1.10 to 1.25 in metacresol was first dried overnight in a vacuum oven at 120°C. The additives were dried at 60°C under vacuum overnight. Concentrates were prepared by first cooling the nylon 612 to 60°C and then tumbling the nylon with additives for 30 minutes end over end. Two concentrates were prepared. The first concentrate contained 90 pounds (40.8 Kg) of nylon 612 and 10 pounds (4.54 Kg) of Additive A. The second concentrate contained 81 pounds (36.7 Kg) of nylon 612,10 pounds (4.54 Kg) of Additive B and 9 pounds (4.08 Kg) of Additive C. Each blend was extruded in a 53 mm twin-screw extruder at 27 pph, with a screw speed of 100 rpm, and a barrel temperature of from 215 to 250°C. The resulting strands were water quenched and cut to flake.

Nylon concentrates of the additives prepared above were blended with additional nylon 612 in the ratios indicated in Table I and then dried overnight at 120°C in a vacuum oven. They were extruded as monofilament through a 1"1-inch (38 mm) single-screw extruder with a screw speed adjusted to maintain constant pressure to a two-capacity Zenith gear pump. The polymer was filtered through five 50-mesh screens and extruded through a .059" (1.5 mm) single-hole die, quenched in water after passage through 8 inches (203 mm) of air. The extruder barrel temperature ranged from 240° to 280°C. The filament was immediately drawn 4X while passing through a steam tube, conditioned for 4 seconds at 180°C, allowed to relax 6% as it came out of the conditioner and then wound on a spool at 860 feet/minute (262 m/min). The tensile properties of the blends were tested, and the results are summarized in Table I.

The filament of Comparative Example B contains 2 weight percent of Additive A, but no aluminum silicate. Comparative Examples C and D are filaments of commercially available nylon 612 and polyethylene terephthalate, without the additives of the present invention.

The filaments were tested by bending four samples of each filament to be tested over a .016" (0.4 mm) steel wire and loading to a tension of 50 grams. The samples are forced against a stainless steel roller turning at 30-35 rpm in at a load of 100 grams/sample. The four samples are kept wet with a 10% slurry of Kaolin in water throughout the test, which lasts 6 hours. Break load and elongation of the four samples are then measured in an Instron tester and the means divided by the unabraded value to obtain percent retention for break load and elongation. The average of these two values is tabulated below:

If the test procedure is repeated, except that the 10% Kaolin is omitted from the water used to wet the samples, the samples will retain at least about 90% of their break load and elongation.

### Examples 10 to 19 and Comparative Examples E to H

The general procedure of Examples 1 to 9 was repeated, except that blends were prepared from three commerically available nylon 66 compositions. Nylon A is substantiate unmodified nylon 66. Nylon B is a copolymer of nylon 6 and nylon 66 blended with about 36% aluminum silicate. Nylon C is nylon 66 blended with about 10% of grafted ethylene alpha-olefin copolymer and 9% of ungrafted copolymer of the types used as Additives B and C in Examples 5 and 6 below. Nylons A, B and C were tumbled and dried in the ratios indicated in Table II. The resulting blends were then extruded as in Examples 1 to 9, except that the melt was filtered through a finer set of screens, the die was 0.95 inches (24 mm) in diameter, and the extruder temperature ranged from 235 to 305°C. The resulting filaments were drawn 2.5 or 3.0 times and conditioned at 220°C. The physical properties of the resulting filaments were evaluated and the results are summarized in Table II.

Comparative Examples E and F were unmodified nylon 66, containing no aluminum silicate. Comparative Example G was unmodified polyethylene terephthalate monofilament. Comparative Example H was a commercially available nylon 66 monofilament containing about 2% of additive A used in Examples 3 and 4 above.

The resulting monofilaments were tested for transverse abrasion as in Examples 1 to 9 above, except that the roller was tool steel rather than stainless steel. Water without Kaolin was used to wet filaments, and the filaments were tested for 3 hours instead of 6 hours. The abrasive used was iron oxide, which accumulated on the roller surface as the test proceeded. It was removed with emery cloth before each new sample was installed. The average retention of break load and elongation after three hours of abrasion is summarized in the following table:

### Example 20

Monofilaments were prepared by direct blending of the components. A blend was prepared by tumbling 142 pounds (64.4 Kg) of nylon 612 for 30 minutes with 51 grams of gamma-aminopropyl triethoxy silane coupling agent. Seven and one-half pounds (3.4 Kg) of aluminum silicate of 1.3 um particle size was added and tumbled for an additional 30 minutes. The blend was then extruded without drying in an 83 mm twin-screw extruder at 141 pounds/hour (63.9 Kg/h) with a screw speed of 130 rpm and a barrel temperature of 255 to 265°C under 6 inches (152 mm) vacuum at the vent port. The molten polymer was fed to eight two-stream, five capacity Zenith gear pumps, filtered through a stack of 33 screens, extruded through a .060" (1.52 mm) single-hole die, and quenched in water after passage through a 4½" (114.3 mm) air gap. The filament was immediately drawn 3.5X in a radiant heater at 840°C, passed through a hot-air conditioning oven at 200°C for 1.4 seconds, and removed from the oven at 40-50 grams tension to cooling rolls after which it was wound on spools at 2070 feet per minute (631 m/min). The monofilament had a caliper of 14.0 mils (356µm).

On testing according to the procedures of Examples 1-9, the filament exhibited a Break Load of 14 pounds (6.35 Kg), an Elongation to Break of 34%, an Initial Modulus of 420 Mpsi (2896 MPa), and a Tensile Strength of 52 Mpsi (359 MPa). The Shrinkage was 6% and the Inherent Viscosity 1.10. The average retention of break load and elongation was 55%.

## Claims

1. An oriented polyamide monofilament having a diameter of from 5 to 30 mils (127 to 762 um) and comprising fiber or filament-forming polyamide and about from 2 to 20 weight precent, based on the total weight of the monofilament, of aluminum silicate having an average particle size of about from 1 to 8 µm.

2. A monofilament as claimed in claim 1 further comprising about from 0.5 to 10 weight percent of an ethylene copolymer having a Melt Index of about from 0.3 to 30 (ASTM D-1238-79).

3. A monofilament as claimed in claim 2 wherein the ethylene copolymer comprises at least about 50% of a graft copolymer prepared from (a) a backbone of polymers selected from the group consisting of thermoplastic polymers of ethylene and copolymers derived from ethylene and C₃ to C₈ alpha-olefins and (b) a graft monomer selected from the group consisting of unsaturated carboxylic acids, anhydrides and dianhydrides.

4. A monofilament as claimed in any one of the preceding claims having a diameter of about from 10 to 20 mils (254 to 508 µm).

5. A monofilament as claimed in any one of the preceding claims wherein the polyamide consists essentially of nylon 66.

6. A monofilament as claimed in any one of claims 1 to 4 wherein the polyamide consists essentially of nylon 612.

7. A monofilament as claimed in any one of the preceding claims wherein the aluminum silicate comprises about from 4 to 10 weight percent.

8. A monofilament as claimed in any one of the preceding claims wherein the aluminum silicate has a particle size such that at least about 90% by weight of the particles are less than 15 µm and the average particle size is about from 1 to 8 µm.

9. A monofilament as claimed in claim 8 wherein the aluminum silicate has a particle size such that 98% of the particles are less than 10 µm and exhibit an average particle size of about from 1 to 6 µm.

10. A woven, heat set, papermaking belt with machine and transverse direction thermoplastic filaments, characterised in that at least about 25% of the filaments in the transverse direction are monofilaments having a diameter of from 5 to 30 mils (127 to 762 µm) and comprising filament forming polyamide and about from 2 to 20 weight percent, based on the total weight of the filament of an aluminum silicate having an average particle size of about from 1 to 8 pm.

11. A papermaking belt as claimed in claim 10 wherein the polyamide monofilaments comprise about from 25% to 50% of the transverse direction strands.

## Patentansprüche

1. Orientiertes Polyamid-Monofil von einem Durchmesser von 5 bis 30 mils (127 bis 762 µm), faser-oder filamentbildendes Polyamid und Aluminiumsilikat von einer durch schnittlichen Teilchengrösse von etwa 1 bis 8 µm in einer Menge von etwa 2 bis 20% vom Gesamtgewicht des Monofils umfassend.

2. Monofil nach Anspruch 1, weiter enthaltend ein Ethylencopolymeres von einem Schmelzindex von etwa 0,3 bis 30 (ASTM D-1238-79) in einer Menge von etwa 0,5 bis 10 Gew.%.

3. Monofil nach Anspruch 2, bei dem das Ethylencopolymere mindestens etwa 50% eines Pfropfcopolymeren umfasst, das hergestellt ist aus (a) einer Hauptkette von Polymeren, ausgewählt aus der Gruppe der thermoplastischen Polymeren von Ethylen und Copolymeren, die von Ethylen und C₃- bis Cₛ-alpha-Olefinen abgeleitet sind, und (b) einem Pfropfmonomeren, ausgewählt aus der Gruppe der ungesättigten Carbonsäuren, Anhydride und Dianhydride.

4. Monofil nach einem der vorhergehenden Ansprüche von einem Durchmesser von etwa 10 bis 20 mils (254 bis 508 µm).

5. Monofil nach einem der vorhergehenden Ansprüche, in dem as Polyamid im wesentlichen aus Nylon 66 besteht.

6. Monofil nach einem der Ansprüche 1 bis 4, in dem das Polyamid im wesentlichen aus Nylon 612 besteht.

7. Monofil nach einem der vorhergehenden Ansprüche, in dem das Aluminiumsilikat etwa 4 bis 10 Gew.% ausmacht.

8. Monofil nach einem der vorhergehenden Ansprüche, in dem das Aluminiumsilikat eine solche Teilchengrösse hat, dass mindestens etwa 90% vom Gewicht der Teilchen kleiner als 15 pm sind und die durchschnittliche Teilchengrösse etwa 1 bis 8 µm beträgt.

9. Monofil nach Anspruch 8, in dem das Aluminiumsilikat eine solche Teilchengrösse hat, dass 98% der Teilchen kleiner als 10 pm sind und die durchschnittliche Teilchengrösse etwa 1 bis 6 pm beträgt.

10. Gewebte hitzefixierte Papiermaschinenbespannung mit thermoplastischen Filamenten in Längs-und Querrichtung, dadurch gekennzeichnet, dass mindestens etwa 25% der Filamente in Querrichtung Monofile von einem Durchmesser von 5 bis 30 mils (127 bis 762 pm) sind und filamentbildendes Polyamid und ein Aluminiumsilikat von einer durchschnittlichen Teilchengrösse von etwa 1 bis 8 µm in einer Menge von etwa 2 bis 20 Gew.%, bezogen auf das Gesamtgewicht des Filamentes, aufweisen.

11. Papiermaschinenbespannung nach Anspruch 10, bei der die Polyamid-Monofile etwa 25 bis 50% der Querstränge ausmachen.

## Revendications

1. Un monofilament de polyamide orienté ayant un diamètre de 127 à 762 µm (5 à 30 mils) et comprenant du polyamide formateur de fibre ou de filament et environ 2 à 20 pour cent en poids, par rapport au poids total du monofilament, de silicate d'aluminium ayant une grosseur de particules moyenne d'environ 1 à 8 µm.

2. Un monofilamenttel que revendiqué à la revendication 1, qui comprend, en outre, d'environ 0,5 à 10 pour cent en poids d'un copolymère d'éthylène ayant un indice de fluidité à l'état fondu d'environ 0,3 à 30 (ASTM D-1238-79).

3. Un monofilament tel que revendiqué à la revendication 2, dans lequel le copolymère d'éthylène comprend au moins environ 50% d'un copolymère griffé préparé à partir de (a) un squelette de polymères choisi dans le groupe constitué des polymères thermoplastiques d'éthylène et des copolymères dérivés de l'éthylène et d'alpha-oléfines en C₃ à Ce et de (b) un monomère de greffage choisi dans le groupe constitué des acides, anhydrides et dianhydrides carboxyliques insaturés.

4. Un monofilament tel que revendiqué à l'une quelconque des revendications précédentes, ayant un diamètre d'environ 254 à 508 pm (10 à 20 mils).

5. Un monofilament tel que revendiqué à l'une quelconque des revendications précédentes, dans lequel le polyamide consiste essentiellement en nylon 66.

6. Un monofilament tel que revendiqué à l'une quelconque des revendications 1 à 4, dans lequel le polyamide consiste essentiellement en nylon 612.

7. Un monofilament tel que revendiqué à l'une quelconque des revendications précédentes, dans lequel le silicate d'aluminium représente d'environ 4 à 10 pour cent en poids.

8. Un monofilament tel que revendiqué à l'une quelconque des revendications précédentes dans lequel le silicate d'aluminium a une grosseur de particules telle qu'au moins environ 90% en poids des particules sont inférieures à 15 um et la grosseur moyenne de particules est d'environ 1 à 8 pm.

9. Un monofilament tel que revendiqué à la revendication 8, dans lequel le silicate d'aluminium a une. grosseur de particules telle que 98% des particules sont inférieures à 10 µm et présentent une grosseur moyenne de particules d'environ 1 à 6 µm.

10. Une courroie tissée, thermo-fixée, pour la fabrication de papier, avec des filaments thermoplastiques dans les directions machine et transverse, caractérisée en ce qu'au moins environ 25% des filaments dans la direction transverse sont des monofilaments ayant un diamètre de 127 à 762 µm (5 à 30 mils) et comprenant du polyamide formateur de filaments et environ 2 à 20 pour cent en poids, par rapport au poids total du filament, d'un silicate d'aluminium ayant une grosseur de particules moyenne d'environ 1 à 8 pm.

11. Une courroie pour la fabrication de papier telle que revendiquée à la revendication 10, dans laquelle les monofilaments de polyamide comprennent d'environ 25 à 50% des brins de direction transverse.
